

L. & H. L. BRADLEY.

TELEPHONE TRANSMITTER.

APPLICATION FILED DEO. 26, 1908. RENEWED JAN. 19, 1914.

1,107,255.

Patented Aug. 18, 1914

Fig. 1.



Fig. 2.



Fig. 3.



Fig. 4.



Fig. 5.

Witnesses:

David S. Gelfish

Wm. Berghahn

Inventors:

Lynde Bradley

Harry L. Bradley

By *Wm. Meiss & Meiss*  
Atlys.

# UNITED STATES PATENT OFFICE.

LYNDE BRADLEY AND HARRY L. BRADLEY, OF MUSKEGON, MICHIGAN, ASSIGNEES TO  
ALLEN-BRADLEY COMPANY, A CORPORATION OF WISCONSIN.

## TELEPHONE-TRANSMITTER.

1,107,255.

Specification of Letters Patent. Patented Aug. 18, 1914.

Application filed December 26, 1908, Serial No. 469,395. Renewed January 19, 1914. Serial No. 813,113.

*To all whom it may concern:*

Be it known that we, LYNDE BRADLEY and HARRY L. BRADLEY, citizens of the United States of America, and residents of Muskegon, county of Muskegon, and State of Michigan, have invented a new and useful Improvement in Telephone-Transmitters, of which the following is a specification.

Our invention pertains to telephone transmitters and particularly to the resistor thereof, viz., to the resistance medium forming a part of the transmitter and serving to vary the resistance of the electrical path through the transmitter in response to the movement of the transmitter diaphragm.

It relates particularly to variable resistances comprising contact elements which vary the resistance of the electrical path in response to changes of pressure.

The mechanism for compressing and relieving the pressure on the resistor forms no part of the present invention, a typical device being shown.

Our invention provides a new resistance element for telephone transmitters of the granular carbon type of construction, our improved substance being utilized for the granular or comminuted material and for the disks or contact faces as well.

Our invention comprises the production of resistance elements which comprise bodies of high conductivity internally and with high contact resistance as a surfacing thereupon. Specifically we prefer to produce a body of carbon in its form of graphite surfaced with carbon in its amorphous form.

In the drawings, Figure 1 shows a complete telephone transmitter; Fig. 2 shows on an enlarged scale the variable resistance parts thereof; Fig. 3 and Fig. 4 show the contact plates or disks, and Fig. 5 shows an alternative form of comminuted material. In the transmitter, which is typical of all the best types of granular carbon transmitters, carbon disks 1 and 2 are soldered or otherwise affixed to metal holders 3 and 4 and comminuted material 5 is placed in the space between these.

In the preferred form of our invention, the disks 1 and 2 are of graphite treated to produce a surface of amorphous carbon. The process whereby we attain this result is as follows: The disks or plates are cut or

sawed from rods of artificial graphite so

that the flat faces are parallel. The plates then are placed in a tray and properly supported so that the flat faces will not make contact with each other. This is done in order that the flat faces all may have free, 60 full and equal access to the solution in which they are to be placed. Then they are immersed in a tank containing coal tar thinned by a "light oil" of the same nature as the tar. The refined coal tar and light oil which we use are obtained as follows: In the processes of making gas from coal, there is produced a "crude coal tar" which, when refined, yields "refined coal tar," "light oil" and other substances. It is the "refined coal 70 tar" and "light oil" thus obtained that we use as a bath in preparing our improved resistance element and our improved resistor. The consistency of the tar and oil bath may be varied as desired. The heavier 75 the bath used, the higher will be the resistance of the resulting resistor. During the first few minutes of immersion the thinning oil enters the plates and leaves a coating of thick tar remaining on the surface, 80 but by the end of about fifteen minutes this sticky coat has been dissolved. After immersion for a sufficient length of time, the disks and the tar mixture are placed in a centrifugal separator and, if necessary, more 85 of the tar mixture is added to insure complete immersion of the disks in the separator. The surplus tar mixture is thrown from the disks centrifugally. The disks then are brushed to remove still further 90 the adhering tar mixture. They are then placed in an oven and kept at 66 degrees C. for about twenty-four hours and again are brushed. This gives them a polish and a smooth surface and tends to prevent sticking together during further baking. They are then packed in tin tubes, placed in an oven and baked at constantly increasing 95 temperatures,—ten hours at 100 degrees C., ten hours at 150 degrees C., ten hours at 200 degrees C., ten hours at 300 degrees C. They are then allowed to cool and are placed in a cast iron retort and are raised to 800 degrees C., which causes a complete carbonization of the tar mixture remaining on 100 and in the disks. Upon cooling they are ready for use. If upon inspection the resistance of any disk should be found too high for the service required, the resistance is lowered by grinding the surface of the 105 110

disk slightly, thus removing a portion of the high resistance coating which the disk acquires by its tar treatment. If the resistance of any disk is not high enough the 5 disk may be subjected to the treatment repeatedly. The disk thus treated may be copper plated upon one of its faces, whereby it may be soldered to its metallic support, 10 or 4.

10 The ability afforded by the foregoing process of producing disks or plates of variant resistances is advantageous, both in the matter of manufacture of the disks and of the comminuted material to be placed between the disks, since it permits the manufacture of transmitter resistance cells whose limiting resistances may be comparatively high or comparatively low. Adopting a musical analogy, the range of the resistor 20 thus may be placed in any selected register.

The production of transmitter resistors of high or low limiting resistances is very important in telephone work. Local battery transmitters for local work operate most 25 satisfactorily with a low resistance; central energy transmitters requiring a higher limiting resistance for local work, and transmitters of both classes operating to better advantage for long distance transmission 30 when built with still higher limiting resistances.

In preparing the comminuted material, the process is substantially the same as for the disks except that the granules or spheres are kept constantly agitated to secure 35 as far as possible an even treatment of their surfaces.

In Fig. 5 a form of comminuted material is shown at 6, which comprises broken sheet 40 material. In the preparation of this material, plates of any convenient size, say an inch in diameter and as thin as can be handled conveniently, say 1/100", are treated on both sides according to the process above 45 described, and then are broken and the fragments sifted through screens to grade them to desired limitations of size. The result is the comminuted material of Fig. 5 which is of value as a resistor for variable resistance 50 compression units such as the telephone transmitter.

Our method of treatment is particularly advantageous in telephone transmitters, because in these resistance units it is desirable 55 that the material forming the resistor shall have a wide range of contact resistance under varying pressure, shall be hard, smooth, polished, capable of carrying a considerable volume of current, having high 60 contact resistance and comparatively low internal resistance of the granules *per se*. It is particularly important in this class of

instruments that the material shall retain these properties permanently so as to prevent the deterioration of the transmitter, 65 and the treated graphite of our invention has proven in experiment and in practice to have such properties.

While we have outlined in this specification with considerable detail the process of manufacture which we have found to be successful, we do not wish to be limited in our claims to the exact details specified, as it is obvious that changes might be made within the skill of one versed in the arts 75 without departing from the spirit of our invention.

Having thus described our invention, what we claim as new and desire to secure by United States Letters Patent is:

1. As a transmitter resistor, two graphite plates surfaced with amorphous carbon and comminuted material therebetween.

2. As a transmitter resistor, two graphite plates surfaced with amorphous carbon and graphite granules therebetween, said granules also being surfaced with amorphous carbon.

3. In a transmitter resistor, a plate of carbonaceous material of high conductivity 90 surfaced with a coating of conducting amorphous carbon, substantially as described.

4. A variable resistor comprising two oppositely placed plates of low resistance carbon surfaced with comparatively high resistance amorphous carbon.

5. In a telephone transmitter, a compressible variable resistor containing a comminuted material, each element of which 100 comprises a graphite body having a surface of carbonized coal tar.

6. In a telephone transmitter, a compressible variable resistor containing a comminuted material, each element of which 105 comprises a conducting body having a carbonized coal tar surface thereon.

7. In a telephone transmitter, a compressible variable resistor consisting of two plates of carbonaceous material and comminuted carbonaceous material therebetween, said plates and said comminuted material each consisting of a body of high conductivity surfaced by a coating of carbonized coal tar.

Signed by us at Muskegon, county of Muskegon and State of Michigan, in the presence of two witnesses,

LYNDE BRADLEY.  
HARRY L. BRADLEY.

Witnesses:

JOHN VANDERWERP,  
JOSIE VANDERWERP.